

## UNITED STATES PATENT OFFICE.

FRANK M. BOYNTON, OF PHILADELPHIA, PENNSYLVANIA.

## RUST-LOOSENING COMPOSITION.

No Drawing.

Application filed July 31, 1925. Serial No. 47,378.

The invention relates to rust loosening compositions particularly intended for use to loosen rusty surfaces as, for instance, the threads of nuts. As is well known to those skilled in the art, nuts, particularly those of large diameter, become rusted to such an extent that it is impossible to remove them unless steps are taken to loosen the rust which has accumulated between the contiguous surfaces. Various rust penetrating compositions have been devised, but the action of these compositions is relatively slow and thereby tends to delay the workman.

I have discovered that a composition containing a proper amount of tetrachlorethane  $C_2H_2Cl_4$  acts on rust with extreme rapidity and is very effective. I prefer to combine the tetrachlorethane with some diluting substance, preferably a liquid hydrocarbon or petroleum derivative, as, for instance, kerosene, varnolene, or similar substances. Preferably the diluting substance consists wholly or chiefly of varnolene, which is a product well known in the art and may be designated as a petroleum fraction free from aromatic hydrocarbons and containing not over 2 per cent of unsaturated hydrocarbons; which petroleum fraction has an initial boiling point between 300° F. and 310° F., a dry or maximum boiling point between 400° F. and 415°

F., a flash point between 105° F. and 115° F., a fire point between 120° F. and 125° F., and a gravity between 49° Bé. and 50° Bé.

The following formula is given as an illustration of a composition which produces excellent results, the proportion given being by weight:—

|                               | Per cent. |
|-------------------------------|-----------|
| Tetrachlorethane $C_2H_2Cl_4$ | 55        |
| Varnolene                     | 35 40     |
| Kerosene                      | 10        |

Such a composition is non-inflammable, relatively inexpensive, and acts with great rapidity.

## What I claim is:

1. A rust penetrating composition which consists of tetrachlorethane and liquid hydrocarbons having a boiling point within the range of that of varnolene and kerosene, said composition being more than half tetrachlorethane, and said liquid hydrocarbons being more than half varnolene.

2. A rust penetrating composition which consists of tetrachlorethane about 55 per cent and varnolene 35 per cent and kerosene 10 per cent.

In testimony whereof I affix my signature.

FRANK M. BOYNTON.